

## UNITED STATES PATENT OFFICE.

AZARIAH Y. PEARL, OF EAST BOSTON, MASSACHUSETTS.

## PROCESS OF DECORATING MATERIAL.

No Drawing.

Application filed August 1, 1922. Serial No. 579,083.

This invention relates to a process of providing material with an iridescent surface and also to material having a decorative surface of this character, and one of the objects of the invention is to provide a novel process by which paper, fabric, celluloid, and a great variety of other material may be provided with an iridescent surface having the characteristic appearance of mother-of-pearl or opal.

Another object of the invention is to provide a novel process of producing this iridescent effect on the surface of material in such a way that the treated material will be entirely non-poisonous and harmless thus making it adaptable for candy boxes, cartons, or containers of food products, covering for toilet articles, etc.

Still another object is to provide a novel process by which the desired iridescent appearance is given to the surface of the material by the deposit thereon of a film, which is transparent and does not, therefore, change the color of the article but which is so formed that in certain lights it has this iridescent or mother-of-pearl appearance.

Still another object is to provide an improved process by which the iridescent film thus deposited produces a water repellent surface and which will become united to the body of the material without the use of adhesive or other binder.

Further objects of the invention will be more fully hereinafter set forth and the novel features of the invention will be pointed out in the appended claims.

As stated above my process may be applied to the decorating of sheet material such as paper, fabric, celluloid, etc., or in fact to a great variety of other material.

In carrying out the process I first apply to the surface to be treated a coating of alum solution, and I will preferably use ammonium alum in forming this solution, although good results can be obtained by using chrome alum or iron alum or other varieties of alum. The alum solution is obtained by dissolving the alum in water and the strength of the solution may be varied within wide limits depending upon the effects desired to be produced.

While the surface to be treated is still wet with this alum solution I expose said surface to fumes of a volatile alkali, such for

instance as ammonia gas and this may be done either in a normal atmosphere or in an atmosphere having an excess of oxygen. I also find that better results are secured when the ammonia gas or other volatile alkali is forced against the wet surface of the material with more or less pressure. The action of the ammonia gas on the wet surface produces aluminum hydrate or aluminum hydroxide in the form of a film, which is deposited on the surface being treated. The formation of this film simulates the formation of frost crystals on window panes, that is the film appears to form progressively and in varied designs. After this aluminum hydrate film has been thus formed the surface may be dried in any suitable way and during the drying the film will become firmly united to the surface.

The film which is formed is transparent so that the natural color of the material is visible therethrough and when the surface is looked at directly the film is almost invisible. If, however, the treated surface is looked at from an angle so that a more or less strong light is reflected toward the observer from said surface at an angle the surface presents an iridescent hue resembling in a marked degree mother-of-pearl or opal. This film which gives this iridescent hue does not contain any pigment or other coloring matter but is apparently in itself transparent although it has the quality of giving the surface an iridescent hue when the surface is observed from the proper angle.

Furthermore this hydrate film is insoluble in water and is tough so that by means of this process the paper, fabric or other material is provided with a tough water repellent surface. The film thus formed is entirely non-poisonous so that the process is adapted for forming decorative paper to be used for candy boxes, containers for food products, etc.

In carrying out the process I find that best results can be obtained when the alum solution is applied to the surface in sufficient quantity so as to form a thin film of solution over the surface at the time that the latter is subjected to the action of the ammonia gas. A fabric or paper surface, when looked at under a powerful microscope will exhibit small fibre ends projecting from the surface and in order to get the best effects it is necessary to have a sufficient thickness of alum

solution covering the surface to submerge or cover these projecting fibre ends. If the fibre ends project through the liquid film they interfere with the crystalline formation of the hydrate film.

The use of iron alum will produce different hues than are produced by the ammonium alum, the iron alum bringing out more of the red hue.

- 10 10. It is also possible to combine my improved process with that of dying or coloring paper. In other words, I may mix the alum solution with a suitable dye which is used for coloring paper and when this is done the action 15 of the ammonia gas on the wet paper will produce the aluminum hydrate film which is deposited on the paper and which acts as a vehicle for the coloring matter or dye so that the dye is deposited with the film. If for 20 instance, a yellow dye is used then the final surface which is produced will be the yellow color with the iridescent hue, or if the paper be treated with a red dye the final product will be a red paper having the iridescent hue.
- 25 25. The decorative surface which is produced by my improved process has a non-metallic iridescent appearance which may be brought out in a great variety of shades and colorings dependent on the character of the 30 aluminum solution used and the character of the volatile alkali.

With my improved process the iridescent hue, which gives the appearance of color, is produced without actually depositing any 35 color on the surface of the article and by means of the deposit of a film which is transparent, and this I regard as one of the distinguishing features of the invention.

I claim:

- 40 40. 1. The process of treating material to produce an iridescent surface thereon which consists in coating said surface with an alum solution and then subjecting said surface to the action of a volatile alkali.
- 45 45. 2. The process of treating material to produce a decorative film on the surface thereof which consists in coating said surface with

an alum solution and then subjecting said coated surface to the action of ammonia gas.

3. The process of treating material to produce an iridescent surface thereon which consists in coating said surface with an alum solution and then delivering ammonia gas under pressure against said surface.

4. The process of treating material to produce an iridescent surface thereon which consists in treating said surface with an alum solution and bringing a volatile alkali in contact therewith.

5. The process of treating material to produce an iridescent surface thereon which consists in treating said surface with an alum solution and bringing ammonia gas in contact therewith.

6. The process of producing an iridescent 65 surface on material which consists in coating said surface with an alum-containing material and then subjecting said coated surface to the action of an alkali thereby to produce a transparent film having an iridescent hue.

7. The process of treating material to provide an iridescent surface thereon which consists in depositing on said surface a film of alum solution and bringing a volatile alkali 75 in contact therewith.

8. The process of treating material to provide an iridescent surface thereon which consists in depositing on said surface a film of alum solution and delivering ammonia 80 gas under pressure against the film.

9. The process of treating material to produce an iridescent surface thereon which consists in forming on said surface a transparent film of aluminum hydrate.

10. Decorative material having a face thereof coated with an aluminum hydrate film.

11. Decorative material having a face thereof coated with an aluminum hydrate 90 film acting as a vehicle for dye material.

In testimony whereof, I have signed my name to this specification.

AZARIAH Y. PEARL.